

# United States Patent [19]

Andres et al.

[11] Patent Number: 4,819,808

[45] Date of Patent: \* Apr. 11, 1989

[54] APPARATUS AND METHOD EMPLOYING MAGNETIC FLUIDS FOR SEPARATING PARTICLES

[75] Inventors: Uri T. Andres, London, United Kingdom; Alan L. Devernoe; Michael S. Walker, both of Schenectady, N.Y.

[73] Assignee: Mag-Sep Corp., Guilderland, N.Y.

[\*] Notice: The portion of the term of this patent subsequent to Jun. 10, 2003 has been disclaimed.

[21] Appl. No.: 869,397

[22] Filed: Jun. 2, 1986

## Related U.S. Application Data

[63] Continuation of Ser. No. 380,753, May 21, 1982, Pat. No. 4,594,149.

[51] Int. Cl. 4 B03B 5/32; B03C 1/00

[52] U.S. Cl. 209/1; 209/214; 209/221; 209/232

[58] Field of Search 209/1, 2, 12, 211, 212, 209/213, 214, 219, 220, 223.1, 232, 172.5, 221, 39, 40; 494/43, 65, 85

## References Cited

### U.S. PATENT DOCUMENTS

|           |         |                     |         |
|-----------|---------|---------------------|---------|
| 653,345   | 7/1900  | Gates               | 209/212 |
| 1,527,069 | 9/1923  | Peck                | 209/214 |
| 2,875,949 | 3/1959  | Tarsoly             | 494/43  |
| 2,967,618 | 1/1961  | Vane                | 209/11  |
| 3,279,602 | 10/1966 | Kottenstette et al. | 209/214 |
| 3,294,237 | 12/1966 | Weston              | 209/214 |
| 3,483,968 | 6/1967  | Kaiser              | 209/1   |
| 3,608,718 | 9/1971  | Aubrey              | 209/214 |
| 3,788,465 | 1/1974  | Reimers et al.      | 209/1   |
| 3,951,789 | 5/1976  | Kaiser et al.       | 209/1   |
| 4,239,619 | 12/1980 | Aplan et al.        | 209/214 |

### FOREIGN PATENT DOCUMENTS

|        |        |          |         |
|--------|--------|----------|---------|
| 78392  | 9/1919 | Austria  | 209/232 |
| 738814 | 7/1966 | Canada   | 209/7   |
| 385623 | 2/1973 | U.S.S.R. | .       |
| 649465 | 2/1979 | U.S.S.R. | .       |

|          |        |                     |       |
|----------|--------|---------------------|-------|
| 831189   | 5/1981 | U.S.S.R.            | .     |
| 1322229  | 5/1973 | United Kingdom      | .     |
| 1497769  | 1/1978 | United Kingdom      | .     |
| 2014062  | 8/1979 | United Kingdom      | .     |
| 7903697  | 8/1979 | United Kingdom      | 209/1 |
| 2064377A | 7/1981 | United Kingdom      | .     |
| 7900622  | 9/1979 | World Int. Prop. O. | .     |

## OTHER PUBLICATIONS

Henry Cohen and Jeremy A. Good, "The Principles and Operation of a Very High Intensity Magnetic Mineral Separator" from IEEE Transactions on Magnetics, vol. Mag-12, No. 5, Sep., 1976, pp. 552-555.

Yehia M. Eissa and Roger W. Boom, "A Feasibility Study Simulating Superconducting Magnetic Separators for Weakly-Magnetic Ores", Journal of Mineral Processing, 2 (1975) pp. 235-248.

(List continued on next page.)

Primary Examiner—Robert B. Reeves

Assistant Examiner—Donald T. Hajec

Attorney, Agent, or Firm—Heslin & Rothenberg

[57] ABSTRACT

A magnetohydrostatic centrifuge of unique geometry in which an elongated separation space is provided within the bore of an elongate cylindrically shaped multipolar magnet. Separations are accomplished both with and without rotation by passing particles to be separated through the separation space within a paramagnetic or ferromagnetic fluid. Certain separations are preferably made using a quadrupolar magnet configuration with a paramagnetic fluid, others with a quadrupolar magnet and a ferromagnetic fluid, and still others, with a sextupolar magnet and a ferromagnetic fluid. Efficient use is made of the magnetic field through the use of a plurality of inner ducts creating a plurality of thin, elongate separation channels characterized by long particle dwell time and short drift distances during the separation process. Significant throughput capacity is achieved in a system in which the magnetic medium is pumped through the separator.

61 Claims, 3 Drawing Sheets



**OTHER PUBLICATIONS**

- P. A. Reeve, "Magnetic Separation in Quadrupole Fields". Proceedings of the International Magnet Technology Conference, Bratislava 1977.
- C. Y. Li et al., "A Superconducting Magneto-Hydromechanical Separator"; IEEE Transactions on Magnetics, vol. Mag-17, No. 1, Jan., 1981.

Soviet Inventions Illustrated, section P4, week E10, Apr. 21, 1982, (London, GB) see abstract 1935E/10,1,99 SU,A,831189.

C. Heck: "Magnetische Werkstoffe und ihre technische Anwendung", Dr. Alfred Huthig Verlag, 1967 (Heidelberg, DE) see page 28, table 1.3.

Magnetohydrodynamic & Magnetohydrostatic Methods of Mined Separation, U. Andres, Keter Publ. House, Jerusalem, Israel, 1976, pp. 13, 163-164.

FIG. 1







**APPARATUS AND METHOD EMPLOYING  
MAGNETIC FLUIDS FOR SEPARATING  
PARTICLES**

This application is a continuation of application Ser. No. 380,753, filed May, 21, 1982, now U.S. Pat. No. 4,594,149.

**BACKGROUND AND SUMMARY OF THE  
INVENTION**

This invention relates to the separation of particulate matter on the basis of differences in magnetic susceptibilities, densities or both.

**DEFINITIONS**

The following terms and phrases are used hereinafter in accordance with the following meanings:

1. Particle to be Separated—Particulate matter, including solids and immiscible liquids.
2. Paramagnetic—Substances, solid or liquid, exhibiting relatively weak positive magnetic properties and which experience forces in a magnetic field which vary in accordance with the product of field strength and field gradient.
3. Ferromagnetic—Substances, both solid and liquid, exhibiting relatively strong positive magnetic properties and which experience forces in a magnetic field which vary only with the field gradient. The term is intended to include ferrimagnetic materials for present purposes because the overall behavior of such materials in our invention is similar to ferromagnetic materials.
4. Diamagnetic—Substances, both solid and liquid, exhibiting negative force proportional to the product of the field and field gradient.
5. Magnetic Fluid Medium—Any fluid substance exhibiting magnetic properties whether ferromagnetic, paramagnetic or diamagnetic. This includes suspensions of magnetic particles in liquids or gases.
6. Elongate—Having length substantially greater than width.

**BACKGROUND OF THE INVENTION**

There has traditionally been great interest in the development of new approaches for magnetic separation, particularly in approaches appropriate for the separation of ores. Major research has been directed towards the development of high gradient magnetic separation (HGMS), a technique which develops an enhanced local magnetic field in the immediate vicinity of a ferromagnetic screen or steel wool. This process is effective for the separation of more weakly magnetic materials than could formerly be treated magnetically, but its application is limited mainly to purification or trace removal requirements. Particles are trapped in the screen and must be washed free, a two-step process not well suited to the separation of large quantities of material as would be required for ores.

Other approaches have involved the further development of new, powerful superconducting magnets for use in direct magnetic attraction of particles using either conventional magnet geometries or new geometries. These direct attraction methods are mainly suited to an extension of the range of conventional magnetic separation to more weakly magnetic particles.

Yet another approach to magnetic separation of ores is known as magnetohydrostatic separation (MHS). Some investigators have concluded that MHS may be

viable for scrap separation, but that its economic application to ore separation is questionable.

Nevertheless, we have discovered a new MHS centrifugal separator and method which permits separation on the basis of small differences in magnetic susceptibilities between even weakly magnetic materials or small differences in density or both. It permits separations which are not now practically feasible to the best of our knowledge. Also, separations can be achieved for very fine particles, even as small as about 1 micron. The throughput capability of our system is considerable and we believe the system can be successfully produced for commercial operation. Our system can operate in a very low range of magnetic susceptibility, a range heavily populated with valuable minerals, which is inaccessible for separation with conventional separation methods.

Briefly described, our system employs a specially designed separation duct surrounded by a multipolar magnet shaped so as to produce substantially only radially directed axisymmetric magnetic forces on materials within the duct. Particles to be separated are passed through the duct in a magnetic fluid medium and undergo radial magnetic forces dependent upon the relative effective magnetic susceptibilities of the fluid medium and the particles themselves. Means are provided for rotating the medium and the particles contained therein in order to create differential centrifugal forces based upon the density differences between the individual particles and between the particles and the medium. Thus, separations can be made without duct rotation on the basis of magnetic susceptibilities only, or they can be made with rotation on the bases of both density and susceptibility differences. Significant rates of throughput are achieved by using a plurality of concentric ducts which, in turn, create a plurality of relatively narrow, elongate annular separation channels. Separation channels of this configuration provide long dwell times as particles travel their length and short drift distances as the particles move radially during the separation process.

Special advantages are available through the use of certain combinations of magnet types and magnetic fluids. More specifically, we have found that the use of cylindrical, open bore quadrupolar magnets in combination with paramagnetic fluids are especially useful for many density separations because this combination in a centrifuge arrangement provides forces on the fluid which increase linearly with radial distance. Thus, separations based on density differences can be made cleanly for particles having magnetic susceptibilities within certain ranges. The same combination of magnet type and magnetic fluid is also particularly useful without rotation for many separations based only on differences in magnetic properties in the particles being separated. Yet, for certain other separations based only on magnetic properties, the combination of a quadrupolar magnet with a ferrofluid medium is more advantageous. We have also found that unique advantages for certain applications are available through the use of cylindrical, open bore sextupolar magnets in a centrifuge using a ferromagnetic fluid. In some cases, the use of a relatively low field strength is most desirable while in others, a relatively high field strength is best. With all of these combinations of magnet types and magnetic fluids, it is, or course, possible to adjust field strength and magnetic fluid properties and, where appropriate, rotational velocities to achieve optimum separation conditions. Further, we believe our new separator design can

be employed in a system in which the magnetic fluid can be passed at sufficiently high rates to produce commercially significant throughput volumes.

The method of our invention is to establish an axially flowing column of a magnetic fluid medium within a magnetic field suitable for producing substantially only radially directed axisymmetric forces on magnetic materials contained within the column. Centrifugal forces may be selectively used for separations where differences in density are present by rotating the column. By means of the interplay of the differential magnetic and centrifugal forces on the particles, various separations can be made in accordance with pre-selected parameters. As noted above, certain separations are optimally made using quadrupolar magnets and a paramagnetic fluid, some being with rotation and other without. Another class of separation is best made with a quadrupolar magnet and a ferrofluid without rotation. Still other separations are advantageously made using a sextupolar magnet in combination with a ferromagnetic fluid in a centrifugal system. Of these, there are some for which the use of relatively low intensity field is appropriate while for others a high field is best.

#### BRIEF DESCRIPTION OF THE DRAWINGS

FIG. 1 is a schematic representation, partly in cross-section, showing an experimental system embodying the invention.

FIG. 2 is an enlarged view of a portion of the separator shown in FIG. 1.

FIG. 3 is a transverse cross-sectional view of the separator taken on line 3-3 of FIG. 2.

FIG. 4 shows an alternate embodiment of the separator duct employing multiple separation channels.

FIG. 5 is a schematic representation showing the manner in which a multipolar electromagnet could be wound for use in our separator.

FIG. 6 is a schematic representation of the magnetic forces experienced by materials within the magnetic fields created by the magnets used in our invention.

#### DETAILED DESCRIPTION OF THE DRAWINGS

FIG. 1 shows an experimental embodiment of our invention in which a special separator duct 10 is centrally located within a cylindrically shaped multipolar magnet 12. A reception funnel 22 is provided for the introduction of ore or other material containing particles 64 and 66 to be separated as well as a magnetic fluid medium 62. Delivery tube 28 delivers the contents of funnel 22 to duct 10. A feed hopper 24 is positioned so that materials to be separated can be fed into funnel 22 in dry or wet form.

Magnet 12 surrounds duct 10 and produces substantially only radially directed axisymmetric magnetic forces on materials contained within duct 10. For purposes of this application, the "separation duct" is understood to mean the duct in which the magnetic field of that character is created and in which the separation of particles takes place. Magnet 12 may be a permanent magnet or an electromagnet having either conventional or superconducting windings. Of course, if a superconducting magnet is used, it would be necessary to encase magnet 12 in a suitable, warm bore dewar, which for present purposes is not shown in FIG. 1. In the case of an electromagnet, the windings may be arranged as illustrated in FIG. 5. There, a quadrupolar magnet 12' is

shown with windings 13 running in elongated longitudinal loops on a cylindrically shaped body 15 having an open central bore 25. Those skilled in the art will appreciate that the magnetic field created by this arrangement, both inside and outside of the magnet, will produce substantially only radially directed axisymmetric forces on materials therein. These forces are illustrated schematically in FIG. 6 wherein the north and south poles are designated by the letters N and S, respectively. The direction of forces experienced upon particles having positive magnetic susceptibilities is indicated by the arrows. Those skilled in the art will also appreciate that for relatively long magnets, where forces are substantially only radially directed throughout most of the magnet length, except for areas near the ends of the magnet. It will also be appreciated that such forces are axisymmetric for a magnet having a cylindrical shape. Although not illustrated, forces of the same character with respect to direction and symmetry can likewise be created with a sextupolar magnet of similar geometry in which north and south poles are alternately arranged around its central axis.

Referring again to FIG. 1, it will be seen that a septum 16 is provided near the lower end of duct 10, duct 10 being shown in a substantially vertical position. The purpose of septum 16, as shown more clearly in FIG. 2, is to physically divide the useful cross-sectional area of duct 10 into inner and outer fraction conduits 13 and 11, respectively. For this purpose, septum 16 is equipped with a knife-edge 17 or other dividing edge at its upper extremity where this physical separation begins.

FIG. 1 also shows a central longitudinal flow guide 14 which is held in place within duct 10 by three vanes 58, more clearly shown in FIG. 3. The purpose of flow guide 14 is to direct the medium 62 and the particles 64 and 66 away from the central portion of duct 10 as those particles move downwardly through the separator. This is desirable because the magnetic and centrifugal forces developed on or about the central axis of duct 10 are either non-existent or so small that they tend to be of relatively little use. By directing the flow of particles into the more outward regions of duct 10, use is made of the stronger forces which are available there in order to make more efficient use of the working volume of magnet 12.

It may be observed in FIG. 2 that outer fraction conduit 11 leads into outer fraction collection tube 18 while inner fraction conduit 13 leads to inner fraction collection tube 19. These tubes are fed into separated product collection containers 38 and 40 illustrated schematically in FIG. 1. There, they are separated from the magnetic fluid medium 62 by any conventional filtering means such as the gravity filtration depicted in containers 38 and 40. The filtering system is desirably effective to sufficiently cleanse and recondition medium 62 so that it may be recycled through lines 54 and 56 as shown. Peristaltic pumps 50 and 52 are provided in lines 54 and 56, respectively, so that the flows can be adjusted in outer fraction conduit 11 and inner fraction conduit 13 for optimum efficiency in accordance with a particular separation being made. The system can, of course, be operated with open flow without recovery and recycling of magnetic fluid 62.

Rotation of the medium 62 and particles 64 and 66 is accomplished in our preferred embodiment by rotation of duct 10 and magnet 12. Vanes 58 are fitted tightly enough inside duct 10 so that flow guide 14 rotates therewith. Septum 16 is rigidly connected to guide 14

and is journaled at its connection with inner fraction collection tube 19. Likewise, duct 10 terminates in an enlarged portion 9 which is journaled at its connection with outer fraction collection tube 18. Rotation is imparted to the assembly by means of drive pulley 32 at the bottom of magnet 12. Drive pulley 32 is connected to a suitable variable speed motor by means of a drive belt, there latter structures not being shown. Reception funnel 22 may be journaled in upper swivel 20 so that it may be restrained from rotating with magnet 12 and duct 10 when desired.

Since the separation duct 10 and the magnetic field created therein are elongate, the particles are given substantial dwell time within the magnetic field so as to provide clean separations even at high rates of flow. An additional advantage of this configuration is that the lateral drift to be negotiated by the particles as they pass through the magnetic field is relatively short. A mathematical description of the separation process in the centrifugal mode of operation and its relationship to duct design is given below.

As shown in FIG. 1, the central axis of the separation duct is vertically oriented. Also, the central axis of the cylindrically shaped multipolar magnet 12 is vertically oriented and coincident with the axis of separation duct 10. In this orientation, the particles can be allowed to fall by gravity through the separation duct.

The invention can be operated in two basic modes, one in which the medium and the particles contained therein are rotated and the other in which they are not. A flowing or stagnant medium and particles can be utilized in either mode.

When the system is operated without duct rotation, separation of particles can be made into two fractions based upon the difference in their magnetic susceptibilities. In this mode of operation, it is necessary to choose a magnetic fluid medium 62 whose susceptibility lies between the magnetic susceptibilities of the two groups of particles to be separated. Under those conditions, particles with a greater susceptibility will be attracted radially outwardly as they pass through separation duct 10, thus becoming outer fraction particles 64 to be collected between septum 16 and duct 10. Particles having a magnetic susceptibility lower than that of medium 62 will be buoyed inwardly and collected within septum 16. It should be noted that if the medium is a ferromagnetic suspension, it will have an effective magnetic susceptibility equal to its magnetization per unit volume divided by the magnetic field strength. This is, of course, true of any ferromagnetic substance.

Additional separations can be made in the other basic mode of operation in which duct 10 is rotated. In this mode, the susceptibility of the magnetic fluid medium 62 is chosen so that it exceeds that of at least some or all the particles to be separated. In this instance, if the susceptibilities of the particles to be separated are reasonably close to one another, separations can be performed on the basis of differences in density. Since some or all of the particles are buoyed inwardly, it is possible to adjust the angular velocity of the duct so that at least some of the heavier particles will be driven outwardly by centrifugal force. In other words, the centrifugal force on these particles will exceed the inwardly directed magnetic buoyancy force on them, if any. By using a relatively weak magnetic field, say about 5000 oersteds (a strong field being about 50,000 oersteds), and a strongly magnetic fluid, the susceptibilities of weakly magnetic particles will have only a small influ-

ence on the separation, and separations based primarily on density differences can be achieved even for particles having significantly different magnetic susceptibilities. The use of a sextupolar magnet, for example, in combination with a ferromagnetic fluid is especially useful in such cases, as will be seen more clearly from the examples given hereinafter.

It should be noted that separation into a plurality of fractions becomes possible in the rotational mode of operation. To accomplish this, it would be necessary to adjust the shape of the magnetic field so as to provide equilibrium positions for particles of various densities.

In either of the above-described modes of operation, the throughput of the system can be increased by causing the medium 62 and particles contained therein to pass downwardly through duct 10. The only limitation on the linear velocity of the medium relates to dwell time. The particles to be separated must have sufficient time in the magnetic field to permit them to be driven to their desired radial positions. Thus, duct 10 is desirably an elongate duct so as to provide adequate dwell times at reasonably high throughput levels.

#### MATHEMATICAL DESCRIPTION OF THE SEPARATION PROCESS IN THE CENTRIFUGAL MODE

The choice of magnet configuration, field strength, angular velocity, and duct design is based upon calculation of the forces to which the particles are to be subjected. These forces, of course, vary with the magnetic susceptibilities and densities of the particles themselves. They are also dependent upon the magnetic properties and the density of the fluid medium.

Consider the case of a paramagnetic fluid in combination with a quadrupole magnet. Let Particle #1 have magnetic susceptibility per unit volume  $\kappa_1$ , density  $\rho_1$  and drag for movement through the fluid,  $D_1$  and Particle #2 with magnetic susceptibility  $\kappa_2$ , density  $\rho_2$  and drag,  $D_2$ . The fluid has density  $\rho_f$  and magnetic susceptibility  $\kappa_f$ . The maximum time required for Particle #1 to move from the inside radius  $r_i$  to the septum (divider) radius  $r_s$  is

$$\tau_1 = \frac{D_1}{F_1} \ln \frac{r_s}{r_i} r_o \quad (1)$$

where

$$F_1 = r_o [\Delta H^2 (\kappa_1 - \kappa_f) + (\rho_1 - \rho_f) \omega^2] \quad (2)$$

$r_o$  is the outside radius of the duct,  $\Delta H$  is the magnetic field gradient, and  $\omega$  is the angular velocity of slurry rotation in radians/sec.

Similarly

$$\tau_2 = \frac{-D_2}{F_2} \ln \frac{r_s}{r_o} r_o \quad (3)$$

for Particle #2 to move from outside radius  $r_o$  to the septum radius, where

$$F_2 = r_o [\Delta H^2 (\kappa_2 - \kappa_f) + (\rho_2 - \rho_f) \omega^2] \quad (4)$$

For best duct design  $\tau_1 = \tau_2 = \tau$  and

$$\omega^2 = \frac{-\Delta H^2 \frac{(\kappa_1 - \kappa_2)}{D_1} + \frac{(\kappa_2 - \kappa_1)}{D_2}}{\frac{(\rho_1 - \rho_2)}{D_1} + \frac{(\rho_2 - \rho_1)}{D_2}} \quad (5)$$

For  $D_1 = D_2$  and minimum  $\tau$ ,  $\tau_1 = \tau_2$  gives

$$r_s = (r_0 \tau)^{1/2} \quad (\text{a condition for duct design}) \quad (6)$$

and

$$\omega^2 = \frac{-\Delta H^2 (\kappa_1 + \kappa_2 - 2\kappa_j)}{(\rho_1 + \rho_2 - 2\rho_j)} \quad (\text{a condition for operation}) \quad (7)$$

For small spherical particles  $D = 18\eta_{\text{eff}}/d^2$ , where  $d$  is the particle diameter and  $\eta_{\text{eff}}$  is an effective viscosity depending upon the solids concentration. The combined vertical flow and drift velocity should be adjusted to allow total particle dwell time,  $\tau_{\text{min}}$ , for the smallest particle and largest  $\Delta\rho$  or  $\Delta\kappa_2$  to be acceptable. That is

$$(v_{\text{flow}} + v_{\text{drift}}) = \frac{L}{\tau_{\text{min}}} \quad (8)$$

where  $L$  is the magnetic field length, and  $v_{\text{drift}}$  is the vertical velocity of the particles relative to the fluid due to gravity.

$$v_{\text{drift}} = \frac{g(\rho - \rho_{\text{fluid}})}{D} \quad (9)$$

The throughput is given by the equation

$$T = A(v_{\text{flow}} + v_{\text{drift}}) \quad (10)$$

where  $A$  is the flow cross-section of the duct. The throughput can be calculated by substitution of (5) into (2), (2) into (1), (1) into (8), and (8) into (10). Analyses similar to the foregoing can be performed for a ferromagnetic fluid and sextupole magnet or other combinations of fluids and multipoles.

From the foregoing, it is clear that particles in a vertically oriented separation duct in which substantially only radially directed axisymmetric magnetic and centrifugal forces are present will be separated into annular fractions. If multipolar magnet 12 is cylindrical shaped, the forces on the particles will depend only on radial position. However, there may be some applications in which "jigging" or the application of a superimposed alternating force would be advantageous. This can be accomplished in a variety of ways. One could, for example, intentionally misalign the separation duct 10 and the magnet 12 with the vertical. Alternatively, one might separate the central axis of the duct from that of magnet 12. A further alternative would be to impart a non-circular shape to the magnetic forces by using ferromagnetic or other suitable materials to reshape the magnetic field somewhat. Or one could simply vibrate the contents of duct 10 via a mechanical "jigging means" (FIG. 1). By doing such things, particles undergoing separation in the rotational mode will experience jigging because of the superimposed cyclically varying forces. It is believed that this would be of advantage in driving the particles through slurries, particularly where the solid loading is high, because the particles

would be jostled about, thus promoting the separation process.

FIG. 4 shows an alternate embodiment of our separation duct which is preferred. Essentially, the purpose of the illustrated structure is to subdivide the useful space within separation duct 10 into a plurality of separation channels 21' and 21''. The reason for doing this is to shorten the radial distance particles must travel in the separation process. The resulting separation channels 21' and 21'' are quite elongate and thin. The relatively long dwell times thus provided, coupled with the short drift distances required for separation, make the separator more efficient, thus making better use of the available magnetic force provided by magnet 12. As shown, outer fraction conduits 11' and 11'' both feed into outer fraction collection tube 18. Similarly, inner fraction conduits 13' and 13'' both feed into inner fraction collection tube 19.

FIG. 4 is intended to be illustrative only. It should be understood that the number of channels like 21' and 21'' might be considerably more than two. Using mathematical analysis like that set forth above, one can compute the optimum number of size of separation channels, considering the loss of useful separation space resulting from the cumulative thickness of the duct walls. Also, we believe that there are alternative means for creating the condition of short particle radial travel under the radial forces by dividing up the space within the duct. For example, one can create a series of concentric annular ducts with small radial thickness. Alternatively, one could construct a single duct comprised of a tightly co-wrapped spiral of inner and outer duct walls and septum. To include this possibility and other divisions of the separation space that accomplish the same end, we refer to such a sub-division of the separator space as "substantially concentric and substantially annular" in the claims which follow.

## EXAMPLES

In the course of our investigation, we constructed two laboratory separators having the general configuration depicted in FIG. 1. A description of these devices is presented in Sections A and B which follow. Separations were performed with these separators on real ores and on two-component mixtures of minerals prepared to simulate different separation problems. Usually the minerals in these mixtures were selected on the basis of distinct color, crystal shape and density differences, so that the separations would be amenable to visual interpretation and results could be clearly presented. Some of the separations of the mixtures are presented in Sections A and B and Table 1, set forth below, as examples of the capabilities of this invention. Note that all results are very good, especially considering that they were each achieved in a single pass of the material through the separator. (Grade and recovery refer to that constituent expected to be mainly present in the inner and outer fraction.)

### A. Separations with the First Laboratory Separator.

The first laboratory separator was constructed using a cylindrical superconducting quadrupole magnet having a 2.75 inch diameter cold bore, an 8-inch useful length and an operating range up to 2.5 Tesla with a 13 kiloGauss per inch gradient. The magnet was located within a 60-inch-long cryogenic containment dewar having an outside diameter of 12 inches and a warm bore of 1-7/16 inches. Several separation ducts were constructed for operation in this device.

The first separation duct was fabricated with a closed bottom from clear polycarbonate. An internal septum was provided for fraction sample collection. In operation, the duct was installed in the warm bore of the dewar and rotated from the top by a variable speed drive motor. Experiments were performed using a static fluid column with hand-feeding of minerals into the top of the delivery tube. The minerals would fall through the fluid approximately 4 feet before they entered the 8-inch-long region of magnet influence of lateral magnetohydrostatic separation forces, reorient themselves radially, and fall into separate concentric collection zones created by the septum.

The results of two of the separations performed with the above apparatus are shown as Examples #1 and #2 in Table 1. The first example illustrates the capability for separation of fine particles by differences in density using our MHS centrifuge. The second example illustrates use of the device in the alternate mode, where separation is achieved by differences in magnetic properties without fluid rotation. To our knowledge, the high quality example separation (of two weakly magnetic minerals having a clear difference in magnetic susceptibility that is small compared to the susceptibility of either constituent) cannot be achieved by any other magnetic separation method, conventional, high intensity or high gradient.

Another separation duct, modified for different presentation of slurry feed into the separation zone, was used to successfully demonstrate separations with a flow of the slurry through the separator using an arrangement like that shown in FIG. 1. This duct provided a thin (1/4-inch-wide) annular flow space for the fluid-particle slurry, demonstrating the separation in a thin elongated separation region. This duct, together with the quadrupolar field configuration and paramagnetic fluid, represents one of the preferred manifestations of the MHS centrifuge concept. One separation in this duct, Example #3, illustrates the ability of our MHS centrifuge to operate with flow of the fluid-particle slurry and to separate materials on the basis of a small difference in particle densities, in this case only 0.5 g/cc. Example #4 illustrates the ability of the device to

achieve quality separations under conditions simulating practical levels of throughput: that is, for a high velocity of slurry flow (33 feet-per-minute) at practical levels of solids concentration (6% by volume). The example here is for the alternate case of separation by differences in magnetic properties, but similar throughputs should result for separations by magnetic properties as well.

Example #5 illustrates that the difficult separation of Example #2 (by weak magnetic susceptibility differences) can also be achieved with a ferromagnetic fluid and under conditions of slurry flow.

#### B. Separations with the Second Laboratory Separator

It became apparent to us that many ores exhibit a variable magnetic characteristic in the concentrate and the gangue that interferes with separation based on density. For these cases, and MHS centrifuge device using a low field is preferred because it is relatively insensitive to the magnetic characteristic of the particles. The stronger, ferromagnetic fluid is also desirable to achieve the inward magnetic buoyancy force levels required. Consequently, a one-meter-long, 2-inch bore MHS centrifuge separator was designed and constructed using samarium cobalt permanent magnets in a sextupolar configuration. The magnets produced 0.398 Tesla at the 2-inch-diameter with a gradient of 7.36 kiloGauss per inch. To save space, the separator was designed so that the magnet assembly would rotate with the duct.

Example #6 provides an illustration of the capability of this device for the type of separation for which it was designed; i.e., density difference separations where variable magnetic characteristics in the concentrate and in the gangue would normally confuse the separation. It is also an example of the use of a sextupole magnet with the ferrofluid, one of the preferred manifestations of our MHS centrifuge concept. A light magnetic mineral was cleanly separated, by density, from a non-magnetic, heavy mineral. Analysis of the separated products shows a 98.5% (Pyrite) grade concentrate and a 5.6% (Pyrite) grade tailing. Recovery of the Pyrite calculates to 98.5% for this separation.

TABLE 1

Examples of Single Pass Separations of Minerals  
Performed with Laboratory Models of the Invention

| Example # and Purpose                                                           | Mineral Mixture                                                                       |                                                                                                 | Fluid Name                        | Magnet Configuration and Construction | Conditions                                       |  | Results                                                         |
|---------------------------------------------------------------------------------|---------------------------------------------------------------------------------------|-------------------------------------------------------------------------------------------------|-----------------------------------|---------------------------------------|--------------------------------------------------|--|-----------------------------------------------------------------|
|                                                                                 | Minerals, Sizes and Amounts                                                           | Densities and Susceptibilities ( $10^{-6}$ emu/cc)                                              |                                   |                                       | Rotation, Field, Field Gradient at Septum Radius |  |                                                                 |
| 1. Sep.* of fine particles by density diff.** (no flow)                         | 33% fluorite<br>44 $\mu$ < d < 74 $\mu$<br>44% < d < 74 $\mu$                         | $\rho = 3.2$ g/cc<br>$\kappa \approx -0.9$                                                      | MnCl <sub>2</sub>                 | Quadrupole, Superconducting           | 180 rpm,<br>3909 Oe,<br>4478 Oe/cm<br>0.87 cm    |  | over 95% recovery and grade in dense and light fractions        |
| 2. Sep. of two weakly magnetic minerals by $\kappa$ (no flow)                   | 50% diopside<br>150 $\mu$ < d < 300 $\mu$<br>50% epidote<br>150 $\mu$ < d < 300       | $\rho = 3.3$ g/cc<br>$\kappa = 28$ to 50<br>$\rho = 3.4$ g/cc<br>$\kappa = 75$ to 116           | Mn(NO <sub>3</sub> ) <sub>2</sub> | Quadrupole, Superconducting           | 0 rpm,<br>3875 Oe,<br>4439 Oe/cm<br>0.87 cm      |  | Over 90% recovery and grade in more and less magnetic fractions |
| 3. Sep. of two materials by small density diff. (flow)                          | ~ 50% aluminum<br>150 $\mu$ < d < 350 $\mu$<br>~ 50% fluorite<br>300 $\mu$ < d < 600  | $\rho = 2.7$ g/cc<br>$\kappa \approx 1.6$<br>$\rho = 3.2$ g/cc<br>$\kappa = 68 \times 10^{-6}$  | MnCl <sub>2</sub>                 | Quadrupole, Superconducting           | 221 rpm,<br>3728 Oe,<br>3358 Oe/cm<br>1.11 cm    |  | 91% aluminum grade in light fraction at 94% recovery            |
| 4. Sep. at high slurry flow (33 ft/min) and solids concentration (6% by volume) | 33% fluorite<br>150 $\mu$ < d < 300 $\mu$<br>67% epidote<br>150 $\mu$ < d < 300 $\mu$ | $\rho = 3.2$ g/cc<br>$\kappa \approx -0.9$<br>$\rho = 3.4$ g/cc<br>$\kappa = 42 \times 10^{-6}$ | MnCl <sub>2</sub>                 | Quadrupole, Superconducting           | 0 rpm,<br>5356 Oe,<br>4325 Oe/cm<br>1.11 cm      |  | Over 90% recovery and grade in more and less magnetic fractions |
| 5. Sep. of two weakly magnetic minerals by $\kappa$                             | 67% diopside<br>150 $\mu$ < d < 300 $\mu$<br>33% epidote                              | $\rho = 3.3$ g/cc<br>$\kappa = 28$ to 50<br>$\rho = 3.4$ g/cc                                   | Aqueous ferromagnetic liquid      | Quadrupole, Superconducting           | 0 rpm,<br>4177 Oe,<br>3764 Oe/cm                 |  | 93% diopside grade with 94% recovery                            |

TABLE 1-continued

| Example # and Purpose                                        | Mineral Mixture                                                           |                                                                                       |                                    |                    | Magnet Configuration and Construction | Conditions                                       |                                             |
|--------------------------------------------------------------|---------------------------------------------------------------------------|---------------------------------------------------------------------------------------|------------------------------------|--------------------|---------------------------------------|--------------------------------------------------|---------------------------------------------|
|                                                              | Minerals, Sizes and Amounts                                               | Densities and Susceptibilities ( $10^{-6}$ emu/cc)                                    | Fluid Name                         | Property and Value |                                       | Rotation, Field, Field Gradient at Septum Radius | Results                                     |
| (flow)                                                       | $150\mu < d < 300\mu$                                                     | $\kappa = 75$ to $116$                                                                | $m = 0.24$ emu/cc                  |                    |                                       | 1.11 cm                                          |                                             |
| 6. Sep. of a magnetic light from a non-magnetic dense (flow) | 60% epidote<br>$74\mu < d < 150\mu$<br>40% pyrite<br>$74\mu < d < 150\mu$ | $p = 3.4$ g/cc<br>$\kappa = 75$ to $116$<br>$\Delta = 5.1$ g/cc<br>$\kappa \approx 1$ | Aqueous<br>ferromagnetic<br>liquid |                    | Sextupole, Permanent Magnet           | 238 rpm, 3480 Oe, 2933 Oe/cm<br>2.38 cm          | 98.5% pyrite recovery in 98.5% pyrite grade |

\*separation;  
\*\*differences

In addition to the foregoing experiments, we have performed other on a similar apparatus which indicate an ability to separate on the basis of small density differences or on the basis of a difference in magnetic susceptibility as small as about  $25 \times 10^{-6}$  emu/cc. Separations have been demonstrated for slurry concentrations of up to 23% solids by weight with fluid flow velocities of up to 33-feet-per-minute.

Our work has demonstrated that it is advantageous to use the combination of a paramagnetic fluid and a quadrupolar magnet for certain density separations and the combination of a ferrofluid and a sextupole magnet for other density separations. Both combinations yield linearly increasing forces on the magnetic fluid medium with radial distance from the axial center to the wall of separation duct 10. The ferrofluid/sextupole combination, however, offers special advantages where separations are to be made on the basis of relatively small density differences in materials having a range of magnetic susceptibilities. As noted earlier, density separations are most easily made when the magnetic susceptibilities of the fractions to be separated are the same, or at least, within a very narrow range. For many applications, the paramagnetic/quadrupolar combination is adequate. But when the range of magnetic susceptibilities becomes somewhat larger, for example, where the spread in susceptibilities is greater than about  $30 \times 10^{-6}$  emu/cc, and where these susceptibilities are spread throughout the gangue of an ore as well as among the valuable minerals to be extracted, it becomes necessary to mask the effects of magnetic susceptibilities. Otherwise, separations will occur on the combined bases of susceptibilities and densities, rather than on the basis of densities alone, as is desired, with the result that the separation would not be particularly clean. With the ferrofluid/sextupole combination, the effective susceptibility of the fluid tends to be higher than that of the constituents of an ore to be separated. Thus, substantial inwardly directed buoyancy forces can be created on all constituents of the ore while selected components thereof can be driven outwardly by centrifugal forces with sufficiently high rotational velocity of the fluid, mainly independent of particle magnetic susceptibilities.

What has been demonstrated by the foregoing is a novel apparatus and method for separating particles in which relatively small differences in density can be used to develop bipolar separation forces at many times the force of gravity. Also, the efficient use of the magnetic field allows the use of less concentrated and less expensive fluids at practical levels of throughput.

A similar advantage results for separation by small magnetic differences in weakly magnetic materials. At the present time, for example, high intensity magnetic separation can only be used to collect minerals having

15 magnetic susceptibilities of about  $200 \times 10^{-6}$  emu/cc or higher, such as wolframite, garnet or chromite. With our separator, however, we can not only collect, but we can actually separate particles from one another on the basis of small differences in magnetic susceptibilities on the order of  $10 \times 10^{-6}$  to  $1 \times 10^{-6}$  emu/cc. Such separations, so far as we know, have not previously been possible and have been regarded by most investigators as unlikely possibilities.

20 The invention described above clearly has broad application, although it may be employed with various modifications. For example, in its rotational mode of operation with flow of the medium, it is not always necessary to orient the separation duct so that its longitudinal axis is parallel with the lines of force in a gravitational field. Also, those skilled in the art will realize that many of the separations described above can be performed outside the cylindrical magnet, although we believe it is more convenient to do so inside. Nevertheless, it is theoretically possible to build an MHS centrifugal separator with its separation channels surrounding the magnet with the use of a diamagnetic field medium. Other modifications can be made concerning rotation of the magnetic fluid medium and the particles contained 25 therein. For example, the vanes 58 on flow guide 14 can be designed in a spiral configuration so that fluid pumped therethrough will undergo a swirling action as it descends through the separator. Also, jiggling might be accomplished by superimposing another magnetic field on the basic field provided by magnet 12. Conceivably, an entirely different magnetic source field could be used in place of magnet 12, the basic requirements being the production of radially directed axisymmetric separation forces without substantial axial components. 30 Clearly, all such designs and modifications are within the spirit of this invention, the scope of which is intended to be limited only by the appended claims.

35 What is claimed is:

1. A method of separating a collection of particles having a range of densities and such magnetic properties as they may possess into two groups of particles based on the combination of each particle's magnetic property and density, the method comprising the following steps:

- 40 (A) establishing along a longitudinal axis and confined within at least part of a surrounding coaxial space a flowing stream comprising the particles to be separated in a fluid medium of positive magnetic property whose density is less than that of all of the particles;
- 45 (B) establishing with respect to substantially the same axis throughout a separation region of said stream a magnetic field with magnitude which decreases

from a point exterior of the flowing stream to the said axis, said field being of such a configuration as to produce substantially only radially directed forces on the medium and the particles;

- (C) rotating the stream about its said axis;
- (D) performing steps (A), (B) and (C) simultaneously while employing a field strength and speed of rotation such that a substantial net radially outward sum of centrifugal and direct magnetic forces exists on all the particles and such that the radially outward attraction of the magnetic fluid by the field provides, additionally, a radially inwardly directed buoyant force on the particles of such magnitude that some of the particles, those having relatively lower combined density and magnetic susceptibility, move inwardly; and
- (E) separately collecting the particles having a relatively lower combined density and magnetic susceptibility as a radially inner fraction and the remaining particles as a radially outer fraction from the stream after it has passed through the separation region.

2. The method of claim 1 wherein the decrease in the magnetic field referred to in step (B) is substantially axisymmetric and radially linear and the fluid medium used in step (A) is paramagnetic.

3. The method of claim 1 wherein the magnetic field establishing step (B) is performed using a quadrupolar magnet surrounding the axis outside the stream and the fluid medium used in step (A) is paramagnetic.

4. The method of claim 1 wherein the magnetic field establishing step (B) is performed using a sextupolar magnet surrounding the axis outside the stream and the fluid medium used in step (A) is ferromagnetic.

5. The method of claim 1 wherein the decrease in the magnetic field referred to in step (B) is substantially axisymmetric and quadratic and the fluid medium used in step (A) is ferromagnetic.

6. The method of claim 1, 3, 4 or 5 wherein the stream establishing step (A) includes the step of forming within the flowing stream a plurality of substreams and wherein the collecting step (E) is performed with respect to each substream.

7. The method of claim 1, 3, 4 or 5 comprising the further step of jiggling the particles to be separated while performing steps (A), (B), (C) and (D).

8. The method of claim 1, 3, 4 or 5 wherein the stream establishing step (A) is performed using a duct and the stream rotating step (C) includes rotating the duct.

9. The method of claim 1, 2 or 5 wherein the magnetic field establishing step (B) is performed using a magnet surrounding the axis outside the stream.

10. The method of claim 9 wherein the rotating step (C) includes rotating the magnet.

11. The method of claim 3 or 4 wherein the rotating step (C) includes rotating the magnet.

12. The method of claim 1, 4 or 5 wherein the effective magnetic susceptibility of the fluid medium used is substantially larger than that of the particles to be separated and the magnetic field strength used is low enough that the forces on the particles due to direct magnetic attraction or repulsion are relatively small as compared with forces due to rotation and magnetic buoyancy.

13. The method of claim 1, 3, 4 or 5 wherein the stream formed in step (A) is annular in cross-sectional shape, at least in the separation region.

14. The method of claim 1, 2, 3, 4 or 5 wherein the collection step (E) includes filtering the particles out of the fluid medium and wherein the fluid medium is then recirculated for repeated use in the method described.

5 15. The method of claim 1 wherein the separation region is elongate.

16. The method of claim 1 wherein the axis is aligned with the lines of force in a gravitational field.

17. A method of separating a collection of particles 10 having a range of densities and such magnetic properties as they may possess into two groups of particles based on the combination of each particle's magnetic property and density, the method comprising the following steps:

(A) establishing along a longitudinal axis and within a confined at least partially surrounding coaxial space a column of a fluid medium of positive magnetic property whose density is less than that of all of the particles;

(B) establishing with respect to substantially the same axis throughout a separation region of said column a magnetic field with magnitude which decreases from a point radially exterior of the column to the said axis, said field being of such a configuration as to produce substantially only radially directed forces on the medium and the particles;

(C) rotating the column about its said axis;

(D) introducing the particles to be separated into the

medium so that they fall through the separation

region;

(E) performing steps (A), (B), (C) and (D) simultaneously while employing a field strength and speed of rotation such that a substantial net radially outward sum of centrifugal and direct magnetic forces exists on all the particles and such that the radially outward attraction of the magnetic fluid by the field provides, additionally, a radially inwardly directed buoyant force on the particles of such magnitude that some of the particles, those having relatively lower combined density and magnetic susceptibility, move inwardly; and

(F) separately collecting the particles having a relatively lower combined density and magnetic susceptibility as a radially inner fraction and the remaining particles as a radially outer fraction from the column after they have passed through the separation region.

18. The method of claim 17 wherein the decrease in the magnetic field referred to in step (B) is substantially axisymmetric and linear and the fluid medium used in step (A) is paramagnetic.

55 19. The method of claim 17 wherein the magnetic field establishing step (B) is performed using a quadrupolar magnet surrounding the axis outside the column and the fluid medium used in step (A) is paramagnetic.

20. The method of claim 17 wherein the magnetic field establishing step (B) is performed using a sextupolar magnet surrounding the axis outside the column and the fluid medium used in step (A) is ferromagnetic.

21. The method of claim 17 wherein the decrease in the magnetic field referred to in step (B) is substantially axisymmetric and quadratic and the fluid medium using in step (A) is ferromagnetic.

65 22. The method of claim 17 wherein the column establishing step (A) includes the step of forming within

the column a plurality of subcolumns and wherein the collecting step (E) is performed with respect to each subcolumn.

23. The method of claim 17 comprising the further step of jigging the particles to be separated while performing steps (A), (B), (C), (D) and (E).

24. The method of claim 17, 18, 19, 20 or 21 wherein the column establishing step (A) is performed using a duct and the column rotating step (C) includes rotating the duct.

25. The method of claim 17, 18 or 21 wherin the magnetic field establishing step (B) is performed using a magnet surrounding the axis outside the column.

26. The method of claim 25 wherein the rotating step includes rotating the magnet.

27. The method of claim 19 or 20 wherein the rotating step (C) includes rotating the magnet.

28. The method of claim 17, 21 or 22 wherein the effective magnetic susceptibility of the fluid medium used is substantially larger than that of the particles to be separated and the magnetic field strength used is low enough that the forces on the particles due to direct magnetic attraction or repulsion are relatively small as compared with the forces due to rotation and magnetic buoyancy.

29. The method of claim 17 wherein the column formed in step (A) is annular in cross-sectional shape, at least in the separation region.

30. The method of claim 17 wherein the column is substantially aligned with the lines of force in a gravitational field.

31. The method of claim 17 wherein the separation region is elongate.

32. Apparatus for separating a collection of particles in a fluid carrier medium having a positive magnetic property and having a density less than that of all the particles, said particles having a range of densities and such magnetic properties as they may possess, into two groups of particles based on the combination of each particle's magnetic property and density, such apparatus comprised of:

(A) means for establishing along a longitudinal axis and confined within at least part of a surrounding coaxial space a flowing stream comprising the medium and the particles to be separated;

(B) means for establishing with respect to substantially the same axis throughout a separation region of said stream a magnetic field with magnitude which decreases from a point radially exterior of the flowing stream to the said axis, said field being of such a configuration as to produce substantially only radially directed forces on the medium and the particles;

(C) means for rotating the stream about its said axis, whereby the particles passing through the separation region experience a net radially outward sum of centrifugal and direct magnetic forces and, in addition, a radially inward magnetic buoyancy force due to the outward attraction of the magnetic fluid by the magnetic field, said buoyancy force being of such magnitude that some of the particles, those having relatively lower combined density and magnetic susceptibility, move inwardly; and

(D) means for separately collecting the particles having a relatively lower combined density and magnetic susceptibility in a radially inner fraction and the remaining particles in a radially outer fraction

from the stream after it has passed through the separation region.

33. The invention of claim 32 wherein magnetic field establishing means (B) is effective to create such a field in which the decrease described is axisymmetric and linear.

34. The invention of claim 32 wherein the magnetic field establishing means (B) is effective to create such a field in which the decrease described is axisymmetric and quadratic.

35. The invention of claim 32 wherein the magnetic field establishing means (B) is comprised of a quadrupolar magnet surrounding the axis outside the confined space.

36. The invention of claim 32 wherein the magnetic field establishing means (B) is comprised of a sextupolar magnet surrounding the axis outside the confined space.

37. The invention of claim 32 wherein the collecting means includes means for filtering the particles out of the magnetic fluid and wherin the invention further includes means for recirculating the fluid back to the stream establishing means for repeated passes through the apparatus.

38. The invention of claim 32 in further combination with positive magnetic fluid for use as a carrier medium in the described apparatus for the particles being separated.

39. The invention of claim 32 wherein the stream establishing means (A) includes means for subdividing the flowing stream into a plurality of substreams, at least within the separation region, and wherin the collecting means is effective to collect radially inner and outer fractions of particles from each substream after it has passed through the separation region.

40. The invention of claim 32 in further combination with means for jigging the particles as they pass through the separation region.

41. The invention of claim 35 or 36 wherein the stream establishing means comprises a duct and the stream rotating means is effective to rotate the duct and the magnet.

42. The invention of claim 32, 33, 34, 35 or 36 wherein the stream establishing means comprises a duct and the stream rotating means is effective to rotate the duct.

43. The invention of claim 32 further comprising a flow guide mounted in the duct by means of vanes tightly engaging the inside surface of the duct.

44. The invention of claim 32 wherein the axis is aligned with the lines of force in a gravitational field.

45. The invention of claim 32 wherein the separation region is elongate.

46. The invention of claim 32 or 45 wherein the stream is annular in cross-sectional shape throughout the separation region.

47. Apparatus for separating a collection of particles in a fluid carrier medium having a positive magnetic property and having a density less than that of all the particles, said particles having a range of densities and such magnetic properties as they may possess, into two groups of particles based on the combination of each particle's magnetic property and density, such apparatus comprised of:

(A) means for establishing along a longitudinal axis and confined within at least part of a surrounding coaxial space a column of a positive magnetic fluid medium;

(B) means for establishing with respect to substantially the same axis throughout a separation region

of said column a magnetic field with magnitude which decreases from a point radially exterior of the column to the said axis, said field being of such a configuration as to produce substantially only radially directed forces on magnetic materials within the region;

(C) means for introducing the particles to be separated into the medium so that they fall through the separation region;

(D) means for rotating the column about its said axis, whereby the particles passing through the separation region experience a net radially outward sum of centrifugal and direct magnetic forces and, in addition, a radially inward magnetic buoyancy force due to the outward attraction of the magnetic fluid by the magnetic field, said buoyancy force being of such magnitude that some of the particles, those having relatively lower combined density and magnetic susceptibility, move inwardly; and

(E) means for separately collecting the particles having a relatively lower combined density and magnetic susceptibility in a radially inner fraction and the remaining particles in a radially outer fraction from the column after they have passed through the separation region.

48. The invention of claim 47 wherein magnetic field establishing means (B) is effective to create such a field in which the decrease described is axisymmetric and linear.

49. The invention of claim 47 wherein the magnetic field establishing means (B) is effective to create such a field in which the decrease described is axisymmetric and quadratic.

50. The invention of claim 47 wherein the magnetic field establishing means (B) is comprised of a quadrupolar magnet surrounding the axis outside the confined space.

51. The invention of claim 47 wherein the magnetic field establishing means (B) is comprised of sextupolar magnet surrounding the axis outside the confined space.

52. The invention of claim 47 wherein the column establishing means (A) includes means for forming within the column a plurality of subcolumns and wherein the collecting means (E) is effective to collect radially inner and outer fractions of particle from each subcolumn.

53. The invention of claim 47 further comprising means for jiggling the particles to be separated as they pass through the separation region.

54. The invention of claim 50 or 51 wherein the stream establishing means comprises a duct and the

stream rotating means is effective to rotate the duct and the magnet.

55. The invention of claim 47, 48, 49, 50 or 51 wherein the stream establishing means comprises a duct and the stream rotating means is effective to rotate the duct.

56. The invention of claim 47 wherein the column is annular in cross-sectional shape, at least in the separation region.

57. The invention of claim 47 wherein the column is substantially aligned with the lines of force in a gravitational field.

58. The invention of claim 47 wherein the column establishing means includes positive magnetic fluid.

59. The invention of claim 47 wherein the separation region is elongate.

60. The invention of claim 47 further comprising a flow guid mounted in the duct by means of vanes tightly engaging the inside surface of the duct.

61. A method of separating a collection of particles having a range of densities and such magnetic properties as they may possess into two groups of particles based on the combination of each particle's magnetic property and density, the method comprising the following steps:

(A) establishing substantially parallel to an axis of rotation and within a confined space a flowing stream comprising the particles to be separated in a fluid medium of positive magnetic property whose density is less than that of all the particles;

(B) establishing within a separation region of said stream a magnetic field with magnitude which increases radially with respect to said axis;

(C) rotating the stream about said axis;

(D) performing steps (A), (B) and (C) simultaneously while employing a field strength and speed of rotation such that a substantial net radially outward sum of centrifugal and direct magnetic forces exists on all the particles and such that the radially outward attraction of the magnetic fluid by the field provides, additionally, a radially inwardly directed buoyant force on the particles of such magnitude that some of the particles, those having lower combined density and magnetic susceptibility, move inwardly; and

(E) separately collecting the particles having a relatively lower combined density and magnetic susceptibility in an inner fraction and the remaining particles in an outer fraction from the stream after it has passed through the separation region.

\* \* \* \* \*